

## UNITED STATES PATENT OFFICE

OSCAR F. MULLER, OF MONTCLAIR, NEW JERSEY, ASSIGNOR TO NYANZA COLOR & CHEMICAL CO., INC., OF NEW YORK, N. Y., A CORPORATION OF NEW YORK

## PROCESS OF DELUSTERING ARTIFICIAL SILK FIBERS OR RAYON

No Drawing.

Application filed May 11, 1929. Serial No. 362,464.

This invention relates to improvements in processes for delustering of artificial silk fibers or rayon. More particularly, this process refers to an improvement in the process 5 shown in my United States Patent No. 1,705,490 of March 19, 1929, relating to the same subject matter.

In the process shown in the patent referred to, I employ an emulsion of olive oil soap in 10 combination with glue and paraffin for a preliminary treatment of the rayon fiber, and then subsequently I subject the fiber so treated with an emulsion to the action of a mild abrasive such as infusorial earth. This process 15 comprises two steps or operations, but I have discovered by further experimentation that by the careful manipulation of my materials rayon or similar fibers may be satisfactorily delustered in a single operation.

20 My improved process is as follows:

First, I prepare an emulsion of paraffin and water with glue and soap as the emulsifying agents; 10 parts by weight of commercial green olive oil soap and 10 parts by weight 25 of medium white glue are dissolved in 100 parts of water. The mixture of soap and glue solution is heated, and then 4 parts of paraffin are added until the paraffin is completely emulsified.

30 I add 2½ parts of the foregoing emulsion to 100 parts of water, and then add to the mixture 5 to 10 pounds of infusorial earth. The mixture is then heated to about 95° F. and is kept at a temperature of from 95° to 35 100° F. during the delustering operation.

The artificial silk or rayon in skein form is put into the mixture and is subjected to the action of this mixture for a period of approximately fifteen minutes. It will be obvious 40 that the duration of the treatment may be varied according to the degree of delustering desired.

Instead of infusorial earth other abrasives may be used, such as chalk, kaolin, fuller's 45 earth, or zinc oxide, and it is also obvious that instead of the specific emulsion mentioned, other liquids may be used to render the surface of the textile fiber receptive to the action of the abrasive.

50 I have found that the abrasive itself is

without permanent effect upon the fiber, unless used in association with a suitable adhesive, as the surface of the fiber is practically unaffected if treated with an abrasive alone.

By the foregoing treatment the process of 55 delustering rayon or similar fibers is much simplified as the entire operation is conducted in a single bath.

Having fully described my invention, what I claim is:

1. A process of delustering artificial silk fibers by subjecting same to the action of an emulsion of paraffin in water having an abrasive suspended therein.

2. A process of delustering artificial silk 65 fibers by subjecting same to the action of an emulsion of paraffin in water having infusorial earth suspended therein.

3. A process of delustering artificial silk 70 fibers by subjecting same to the action of an emulsion of a colloidal material having an abrasive suspended therein.

4. A process of delustering artificial silk 75 fibers by subjecting same to the action of an emulsion of a waxy material having an abrasive suspended therein.

5. A process of delustering artificial silk fibers by subjecting same simultaneously to the action of a bath containing a wax emulsion and abrasive substance.

6. A process of delustering artificial silk 80 fibers by subjecting same simultaneously to the action of a bath containing a wax emulsion and infusorial earth.

7. A process of delustering artificial silk 85 fibers by subjecting same simultaneously to the action of a bath containing an emulsion of paraffin and infusorial earth.

8. A process of delustering artificial silk 90 fibers by treating same with an emulsion having an abrasive suspended therein.

9. A process of delustering artificial silk fibers by treating same with an emulsion having infusorial earth suspended therein.

10. A process of delustering artificial silk 95 fibers by treating same with an emulsion containing glue and paraffin and having an abrasive suspended therein.

11. A process of delustering artificial silk 100 fibers by treating same with an emulsion con-

taining glue and paraffin and having infusorial earth suspended therein.

12. A process of delustering artificial silk fibers by subjecting same to the action of an emulsion containing glue and paraffin, said emulsion having an abrasive suspended therein at a temperature of from 95-100° F.

13. A process of delustering artificial silk fibers by subjecting same to the action of an emulsion containing glue and paraffin and an abrasive for a period of fifteen minutes at a temperature of approximately 95-100° F.

In testimony whereof I affix my signature.  
OSCAR F. MULLER.

15

20

25

30

35

40

45

50

55

60